

## UNITED STATES PATENT OFFICE

PHILIP W. CODWISE, OF KENMORE, NEW YORK, ASSIGNOR, BY MESNE ASSIGNMENTS,  
TO CERTAIN-TEED PRODUCTS CORPORATION, A CORPORATION OF MARYLAND

## FELT

No Drawing.

Application filed July 8, 1925. Serial No. 42,316.

This invention relates to a method of preparing an absorbent material and to a product which can be used advantageously as a foundation for materials for roofing, floor covering, insulating, sheathing and the like. The material is especially porous and absorbent and is adapted, therefore, to be saturated or impregnated with a waterproof composition and to receive coatings such as asphalt or pitch. It has also sufficient strength to withstand the strains to which it is subjected in saturating tanks, squeeze rolls, and other mechanical devices.

This application is a continuation in part 15 of my copending application Serial No. 21,727, filed April 8, 1925 and also contains features which are disclosed in my co-pending application Serial No. 130,361, which is a continuation in part of said application, Serial 20 No. 21,727, filed April 8, 1925, and of this present application.

Roofing felt has been made heretofore almost exclusively from rag stock because no other satisfactory material has been available 25 for that purpose. The supply of rag stock is limited and it is, therefore, comparatively expensive. To reduce the cost, there is sometimes used ordinary paper or wood pulp, whether produced by mechanical or chemical 30 disintegration, consisting essentially of ultimate fibres of cellulose which are much too fine to possess the necessary absorbent properties for asphalt or pitch. Such fibres mat readily into a dense mass which lacks porosity, 35 the resulting sheets being entirely different in character from the porous felt required in industries wherein properly saturated and water-proofed bases must be used. The usual addition of paper pulp to rag stock to produce 40 a satisfactory felt is about 10% but such an addition does not reduce the cost sufficiently to offset the inferior saturating qualities resulting.

It is the object of the present invention to 45 provide a cheaper and more satisfactory felt material for the purpose mentioned, which saturates more readily than ordinary rag felt, or rag and paper felt. The material is derived from wood but it is entirely different 50 in nature and properties from ordinary pa-

per or wood pulp, mechanical or chemical, and possesses the necessary characteristics to ensure absorption of saturating materials and thus to provide a suitable foundation for roofing, floor covering or similar bases.

Other objects and advantages of the invention will be apparent when reference is had to the following specification in which the preferred embodiments are described to exemplify the method and product.

I have discovered that a satisfactory felt-ing material can be prepared by suitably treating wood chips so that the resins and lignins therein are only partially removed, leaving the fibre in the form of bundles cemented together by the natural contents of the wood. These bundles are to be distinguished from the ultimate fibres such as are obtained in the manufacture of the usual chemical wood pulp, since they can be 65 formed into a felt having great porosity and capillary attraction for molten saturating or impregnating material as well as high tensile strength. Various woods may be utilized in preparing the fibre bundles but the so-called 70 coniferous woods, such as pine, fir, hemlock, cedar and spruce are especially satisfactory sources of the material because of the length and other characteristics of the fibres incorporated therein.

To prepare the material the wood is chipped in the usual log chipper or similar machine. Preferably the chips are subjected to a preliminary steaming in any suitable apparatus to soften the binding material and are then impregnated thoroughly with an alkaline solution containing for example, sodium hydroxide. The impregnated chips are then cooked in the alkaline solution with steam at an elevated temperature and pressure until the desired effect is obtained. This is accomplished when the chips are so digest-ed that they can be disintegrated readily 80 into masses of long fibre bundles which when washed and beaten in water intertwine and 85 felt. It is important to note that the opera-tion must be conducted to avoid disintegra-tion into ultimate fibres as is the case in the manufacture of paper pulp. While it is pref-90 erable to first steam and impregnate the chips, 95 in nature and properties from ordinary pa-

these steps can be omitted, the cooking being conducted direct with steam as soon as the alkaline solution has been added to the chips. In such case the operation is slower but substantially the same results are obtained.

When the chips are removed from the digester they are apparently in their original physical condition but in fact they have undergone an important change as they are soft and spongy and the fibres have acquired remarkable capillary properties which are not noticeable in the uncooked wood. The treatment with alkaline solutions removes a moderate amount of resins and lignins, and softens the remaining material which originally bonded the fibres together. Thus the bond between the fibre bundles is loosened without disintegrating the mass into the ultimate cellulose fibres. The loosening of the bond facilitates the separation of the fibre bundles so as to render them suitable for processing in accordance with the steps hereinafter to be referred to. When separated the bundles are soft and fluffy and can be felted after beating to produce a strong and porous sheet.

As an example of the method herein disclosed 100 parts of pine wood chips of approximately 1" in length are placed in a digester and steamed for approximately  $\frac{3}{4}$  of an hour. The chips are then impregnated in the digester under a pressure, preferably up to 100 pounds per square inch, with an excess of sodium hydroxide solution of 5% or less concentration. The impregnation period during which the chips are thoroughly impregnated continues for approximately  $\frac{3}{4}$  of an hour when the excess liquid is drawn off to be reused on subsequent batches. Only a sufficient quantity for cooking purposes now

40 remains in the chips so that the dry weight of sodium hydroxide present, equals 14% or less of the dry weight of the wood chips. The amount of sodium hydroxide used in cooking will vary somewhat with the nature of the wood, especially with the resin content of the wood, but will seldom be below 4% or above 14%. Following the impregnating period, steam is allowed to enter the digester until the temperature rises to approximately 50 160° C.; the pressure during this period ranging from 60 to 120 pounds per square inch. This is known as the cook period and continues from 3 to 5 hours, depending on the nature of the chips used. When the cook period has been completed, the cooked chips are removed from the digester and washed. The chips are then partly disintegrated, shredded or torn apart by any mechanical means into fibrous bundles, washed and beaten slightly with water and thereafter made into a sheet by any known felting apparatus. An ordinary paper machine as used at present in felt manufacture, such as the cylinder or Fourdrinier type is suitable for this purpose.

If desired the operation described above can be condensed into a single operation which produces the same result, but is somewhat more time consuming. This is to place 100 parts of wood chips in a digester and immediately add thereto approximately 250 parts by weight of water and about 8 parts by weight of sodium hydroxide. The entire mass is immediately cooked under pressure of 60 to 120 pounds per square inch at a temperature of approximately 160° from 5 to 12 hours. The chips are then ready to be disintegrated and treated as described above. The proportion of sodium hydroxide used in this method will vary from 4%-14%, depending upon the wood used.

Any type of wood which will soften and develop absorptive properties when treated with alkaline solutions at elevated temperatures, is suitable for the purpose of this invention, but it is preferred to use coniferous wood, especially pine, because of its suitability and low cost. Any alkaline solution which will soften the wood and develop absorptive properties in the same is suitable for the purpose of this invention, but it is to be understood that the invention is not to be limited to the use of sodium hydroxide. Alkaline solutions of sodium sulphite have produced similar results and other alkaline solutions, such as sodium carbonate, calcium hydroxide and the like can be used in combination with similar results. The proportion of water to the chips may be varied according to the material used.

The method produces a sheet of sufficient strength and pliability to be rolled and treated as is usual in preparing saturating felt. The sheet possesses high capillarity not only by virtue of the voids formed in the fibres themselves, but also by virtue of the formation of numerous voids between the fibre bundles resulting in high absorptive characteristics in the product. The cooking process is essential for the production of such capillarity and of pliability in the product, and the disintegration or tearing apart of the fibre bundles with water is desirable for the production of satisfactory bonding of the fibre bundles and the production of satisfactory tensile strength in the product. Material prepared as herein described produces a sheet which will absorb saturants at a more rapid rate and to a much higher degree than fibrous material obtained from ordinary pulp. A sheet made according to the described method is composed of long absorbent fibres which in addition to their absorptive qualities, due to their length, will interlock causing numerous openings there-between for quick penetration of the saturating material. The felt made according to this invention may moreover absorb 300% or more of its weight of roofing asphalt as compared with the ordinary rag felt which

usually absorbs only 180% or less of its weight.

The fibrous sheet material made as herein described may be too absorbent for some purposes, and to retard the absorption, rag fibres or waste paper may be intermixed when feltting the sheet. The quantities of the various fibres used depends upon the intended purpose and use of the material.

10 Matter not claimed in this application is made part of and claimed in my co-pending applications Serial Numbers 130,361 and 130,362 filed August 19, 1926.

Obviously the present invention is not restricted to the details of the particular embodiment thereof herein described. Moreover, it is not indispensable that all the features of the invention be used conjointly since they may be employed advantageously in various combinations and sub-combinations.

Having described one embodiment of the invention I claim:

The method of making felt which comprises preliminarily steaming wood chips, impregnating the same under pressure with excess of sodium hydroxide solution of 5% or less concentration, draining off the liquor after impregnation to an extent to leave an amount containing 4% to 14% of alkali in relation to the weight of the chips, cooking the chips with this liquor under pressure under such conditions as to soften them and incompletely release the bond between the fibres to maintain the fibres in their natural positions in the chips, and then shredding the chips to separate the same for the most part into bundles of the fibres, and matting the same into sheets.

In testimony whereof, I affix my signature.

40 PHILIP W. CODWISE.

45

50

55

60

65